

3,827,882

**HIGH LEAD ALUMINUM ALLOY**

Kenneth Lloyd, Chesham and Anthony Dennis Michael, London, England, assignors to The Glacier Metal Company Limited.

No Drawing. Continuation of application Ser. No. 807,425, Mar. 14, 1969. This application Sept. 24, 1971, Ser. No. 183,705

Claims priority, application Great Britain Mar. 15, 1968, 12,785/68.

Int. Cl C22c 21/00

U.S. CL. 75—138

3 Claims

**ABSTRACT OF THE DISCLOSURE**

This invention is a bearing alloy for acting as a lining on a steel backing. Good bearing properties are given by having a high percentage, preferably between 10% and 12% by weight, of lead in aluminium. Strength can be given by some silicon and some calcium improves the solubility of the lead in the aluminium and up to 1% of lithium may be added to globularize the lead in the aluminium.

This is a continuation of application Ser. No. 807,425 filed Mar. 14, 1969, now abandoned.

This invention relates to an aluminium base alloy particularly for use as a bearing material, for example in thin shell bearings where the alloy requires to be bonded by rolling to a steel backing either directly or with an intermediate layer of metal foil, or after the backing has been plated with say nickel or cobalt.

According to the present invention, a bearing alloy which may be bonded to a steel or other backing, comprises aluminium and more than 3% of lead by weight. Perhaps there may be 10%—20% of lead, and preferably 10%—12%.

It has been discovered that such a bearing has a surprising ability to survive without pick-up or seizure, momentary contact with the journal when for any reason the oil film thickness becomes locally less than the surface roughness. This property is known as compatibility. While softness of the material is a factor in obtaining this property, other factors are relevant, and the property is, in general, little understood.

According to a feature of the invention an aluminium base alloy, suitable for use as a bearing alloy and capable of being bonded to a steel backing, contains by weight 0.5% to 11.3% silicon and by weight from 3% or 3.2% to 26% lead, the balance being aluminium except for normal impurities and from 0 to 1% of each of one or more of the elements copper, nickel and manganese to improve the strength of the aluminium matrix, and from 0 to 3% of calcium to increase the solubility of the lead in the aluminium. It would probably be necessary to have a much higher proportion of calcium in the melt in order to get 3% in the casting, because much calcium would be evaporated off at the necessary temperature of the melt.

The silicon gives strength to overcome the effect of the high proportion of lead, but the maximum amount of silicon in the alloy should be not more than about 12% by weight of the aluminium present, so that the alloy remains *hypo-eutectic* in structure. That is to say that since the silicon is almost solely contained in the aluminium phase, if the lead content by weight were 20%, the total silicon content should not exceed 9.6% by weight in the alloy otherwise the alloy could be *hypo-eutectic* and subsequent roll bonding of the material would be exceedingly difficult, if not impossible.

The silicon is present preferably as a proportion of 0.5% by weight of the alloy, in order to increase the

strength, hardness, and wear resistance, properties of the alloy as well as reducing its tendency to seizure and may increase the lead at which scurfing occurs.

The lead provides the surface properties required of a bearing alloy, but preferably the whole alloy is of uniform composition, and is not of the defined composition at the bearing surface.

The aluminium base alloy according to the invention may contain a small addition of tin to the alloy. The lead phase in an aluminium-lead-silicon alloy is almost pure lead since the solubility of silicon and aluminium in lead are very low. Pure lead is particularly prone to corrosive attack especially by organic acids such as may be present in the lubricating oil of a plain bearing. The corrosion resistance of lead can be greatly improved by additions of small amounts (up to 6% by weight) of tin.

Accordingly this invention provides for an addition of tin such that the amount of tin in the lead phase is up to 6% and preferably 3%. Since the solubility of tin in aluminium and silicon is extremely low, any addition of tin is almost entirely dissolved by the lead phase. Thus, to obtain a tin content of 3% by weight in the lead phase a total addition of only 0.3% need be made to the complete alloy containing 10% of lead by weight.

An alloy according to the invention may also include up to 1% by weight of the whole alloy of bismuth, and this will reduce the ductility of the lead and the lead and the tendency, when the alloy is roll bonded to a steel backing, to form long stringers of lead. The addition of bismuth will cause these lead stringers to break up when the material is rolled. Tellurium may replace bismuth with a similar effect. Up to 1% by weight of the total alloy of cerium or lithium may be added to "globularize" the lead in the aluminium.

The invention includes a bearing comprising a layer of an alloy as defined, and also a layer of the alloy bonded to a steel or other backing.

That aluminium-lead alloys have not been developed earlier for use as bearing alloys is due to the technical difficulties imposed on their manufacture by the abnormal configuration of the equilibrium diagram of aluminium-lead and the large difference in their densities.

When the lead content in aluminium exceeds 2% by weight, during casting the alloy passes through a temperature range where the aluminium and lead molten liquids are completely immiscible in one another and as a result of the large density difference the lead sinks rapidly to the bottom. To achieve a homogeneous alloy, it may be necessary during casting to extract the heat from a vertical length of the solidifying alloy at such a speed that the alloy solidifies very rapidly so as to minimise the time to pass through this temperature range. Such a process is possible, although difficult, on a small scale by producing chill castings in a mould arranged in such a way as to cause the heat to be extracted vertically (i.e. not through the walls of the mould) and rapidly. An easier and more reliable method has been developed. Patent Application No. 519,096, now Pat. No. 3,432,293 discloses a continuous casting method in which the alloy is introduced into the mould at a temperature at which aluminium and lead liquids are miscible and in which the melt is solidified rapidly creating a substantially vertical temperature gradient such that the solidification isotherms are substantially horizontal and hence prevent the segregation in a vertical plane. Such a method is capable of producing aluminium-lead alloys of high lead content uniformly and evenly dispersed as fine particles in the alloy. The addition of silicon to the alloy made for reasons of improved bearing properties also effects an improvement in the surface quality and lead distribution in billets made by this method. The fineness of the lead particles, which is im-

portant for a bearing material, is dependent on the speed at which the alloy is chilled from the homogeneous liquid through the two-immiscible-liquids region.

The invention may be carried into practice in various ways but two alloys will be quoted by way of example.

#### EXAMPLE I

The alloy was constituted of:

|           | Percent by weight |
|-----------|-------------------|
| Lead      | 10                |
| Silicon   | 4                 |
| Copper    | 1                 |
| Tin       | ½                 |
| Calcium   | ½                 |
| Aluminium | Balance           |

#### EXAMPLE II

|           | Percent by weight |
|-----------|-------------------|
| Lead      | 12                |
| Copper    | 1                 |
| Tin       | ½                 |
| Silicon   | ½                 |
| Aluminium | Balance           |

In each case, the cast alloy had reasonable distribution of the lead without its collecting into too large local

"pools." The bearings had long life with little wear and without seizing.

What we claim as our invention and desire to secure by Letters Patent is:

5 1. In an aluminum-lead bearing alloy consisting essentially of aluminum and from 10 to 26 wt. percent of lead, the improvement which consists in including therein lithium in an effective amount up to 1% by weight of the total alloy to globularize the lead in the aluminum.

2. A bearing alloy member capable of being bonded to a steel backing and consisting essentially of aluminum, lead and lithium, the content of lithium being present in an effective amount up to 1% of the total alloy and sufficient to globularize the lead in the aluminum, the content of lead being from 10 to 26% by weight of the alloy.

3. A bearing alloy as claimed in Claim 1 including 0.5% of silicon.

#### References Cited

##### UNITED STATES PATENTS

20 3,545,943 12/1970 Miller et al. ----- 75—138  
1,620,082 3/1927 Czochralski ----- 75—138

RICHARD O. DEAN, Primary Examiner

25 U.S. CL. X.R.

75—139, 140, 143, 148